

Dec. 22, 1925.

1,566,749

W. G. IMHOFF

APPARATUS FOR USE IN HOT GALVANIZING AND THE LIKE

Filed April 16, 1923



INVENTOR  
Wallace G. Imhoff  
by William T. Orrharton  
his attorney

Patented Dec. 22, 1925.

1,566,749

# UNITED STATES PATENT OFFICE.

WALLACE G. IMHOFF, OF PITTSBURGH, PENNSYLVANIA, ASSIGNOR TO WARREN S. SMITH, OF NEW YORK, N. Y.

## APPARATUS FOR USE IN HOT GALVANIZING AND THE LIKE.

Application filed April 16, 1923. Serial No. 632,197.

To all whom it may concern:

Be it known that I, WALLACE G. IMHOFF, a citizen of the United States, residing at Pittsburgh, in the county of Allegheny and State of Pennsylvania, have invented a new and useful Improvement in an Apparatus for Use in Hot Galvanizing and the like, of which the following is a specification.

This invention relates to apparatus for use in hot galvanizing, and to a method of protecting galvanizing apparatus and other articles from the action of molten zinc.

In the process of hot galvanizing the articles being galvanized are passed through a bath of molten zinc maintained at a temperature of approximately 820 degrees Fahrenheit to 950 degrees Fahrenheit. Such bath usually contains a small percentage of certain other metals, such as tin, antimony, and aluminum. This bath is contained in a vessel, known in the trade as a galvanizing kettle, the sides of which are commonly made of fire-box steel and the bottom and ends of flange steel, or boiler steel. A part of the permanent equipment is a thermometer, or pyrometer, for taking the temperature of the bath. This is enclosed in a casing which extends below the surface of the molten zinc.

The great difficulty encountered in the process of hot galvanizing is that the molten zinc gradually dissolves any metal with which it is in contact for any length of time, forming a zinc alloy known as "dross."

It is further a fact that molten zinc is possessed of highly penetrative properties, so that it permeates the pores, or microscopic apertures, in a metallic body. As the dross itself when formed furnishes no protection to the still unattacked body of metal, the action of the molten zinc is progressive, terminating only with the complete destruction, or dissolution, of the body with which it comes in contact.

The dissolving action of the zinc involves a great loss in the destruction of the galvanizing kettles, which are necessarily expensive, and in the destruction of the pyrometer tubes which contain the thermometer or thermo-couple for regulating the temperature of the bath. For this reason extensive experiments have been carried out for the purpose of discovering a metal, or metallic alloy, which would not be attacked by molten zinc. With this object in view experiments were made with nickel, Monel

metal, duriron, calite, resistal, ferralt, wrought iron, cast iron, all kinds of steel, and with substantially all ferrous and other alloys in common or scientific use. All metals and all alloys tested, however, were found to be attacked in varying degrees by the molten zinc. The fact that certain alloys were capable of resisting oxidation or attacks by various acids has proven to be no criterion of their ability to resist the attacks of molten zinc.

Various coatings applied to the metal as by japanning, calorizing, or parkerizing the same have also proven of no value in protecting the metal from the molten zinc.

The object of the present invention is, therefore, to provide metallic articles, particularly galvanizing kettles and thermometer and pyrometer casings with a coating capable of effectually protecting the same from the dissolving action of molten zinc.

I have succeeded in effecting this purpose by applying to the metallic articles a protective coating having a silicious base. I have discovered that certain silicates, and particularly boro-silicates, are not subject to attack by molten zinc. In forming such a coating I apply to the interior surface of a galvanizing kettle or to the exterior surface of a thermometer or pyrometer casing, one or more coats of a highly silicious or "refractory" enamel, which has also a very dense or highly glazed or "vitreous" surface. Such coating serves as an impermeable medium interposed between the metal of the article and the bath, and which is itself unaffected by the action of the molten zinc.

The accompanying drawings show in cross section a galvanizing kettle and thermometer tube provided with the protection of the present invention.

In such drawings the reference numeral 1 designates the usual refractory setting for the kettle, 2 the draft apertures through such setting, and 3 the filling of coke which is burned to heat the kettle and the zinc which it contains.

The galvanizing kettle is shown as constructed in the usual manner with sides 4 of relatively thick plates of fire box steel, and with ends and bottom 5 of flange steel secured to the sides by rivets or the like. A tubular casing 6, provided with a thermometer 7, is shown projecting downwardly into the body of the kettle. The interior surface

2  
of both the sides, bottom, and ends of the kettle is provided with a protective coating 8 of enamel.

The preferred enamel for this purpose is one of a highly refractory character, having a highly glazed or vitreous surface. The principal components of such enamel are silica and boric oxide, combined with alumina and other oxides as calcium oxide, sodium oxide, potassium oxide. The relative proportions of these components may be varied within relatively wide limits, but I prefer those mixtures which are baked on at from 1000 degrees Fahrenheit to 1500 degrees Fahrenheit, and which give a highly glazed surface. It may be stated as a general rule that the percentages of silica and boric oxide in the enamel should be so proportioned as to impart a smooth glaze to the enamel coating. Such mixture comprising silica, boric-oxide, and alumina, together with one or more other oxides, results in the formation of an enamel comprising a complex aluminum boro-silicate as a basis thereof. 25 The coat of enamel may be applied to the interior surface of the galvanizing kettle by painting, dipping, spraying, dusting, or in any usual manner of applying such coatings, and is baked on in the usual manner at the requisite temperature. A plurality of coats may desirably be applied in building up the complete coating. The exterior surface of the thermometer or pyrometer casing is provided with a similar coating of enamel, 35 which is similarly baked on.

It has been proved that such coating is effective in protecting metals from the attacks of molten zinc; and such effectiveness may be attributed to the fact that the silicates forming its chief component are not themselves subject to the solvent action of molten zinc at galvanizing temperatures, and to the fact that the glazed surface of the enamel is capable of resisting the penetrative action of the molten zinc. It will be readily appreciated from the composition of the enamel employed, that a coating of the same constitutes a good heat conducting medium. It does not, therefore, retard the melting of spelter in a galvanizing kettle, or impair the functioning of a thermometer immersed in the bath.

It will be understood that the method of protecting articles from the attacks of molten zinc may be utilized for other pur-

poses than the protection of galvanizing kettles and the thermometer and pyrometer casings used therewith. For example a similar protective coating may be applied to molds for casting zinc slabs at the smelters, 60 and to the interior surface of tubes for conveying molten zinc, or for other similar purposes.

What I claim is:

1. Apparatus for hot galvanizing and the like comprising a galvanizing kettle having a body of ferrous metal, and a coating of an enamel comprising a complex aluminum boro-silicate as the basis thereof on the interior surface of the body of the kettle, to 70 provide a heat conducting medium for protecting the same from the solvent action of molten zinc contained in the kettle.

2. In apparatus for use in hot galvanizing and the like, an article to be brought into 75 contact with molten zinc comprising a metallic body, said body having a coating of an enamel comprising a complex aluminum boro-silicate as the basis thereof on the surface of the body which comes into contact 80 with the molten zinc to provide a heat conducting medium for protecting the body of the article from the solvent action of the molten zinc.

3. In apparatus for use in hot galvanizing 85 and the like, an article to be brought into contact with molten zinc comprising a metallic body, said body having a coating of an enamel comprising a complex aluminum boro-silicate as the basis thereof together with boric-oxide on the surface of the body which comes into contact with the molten zinc to provide a heat conducting medium for protecting the body of the article from the action of the molten zinc. 95

4. In apparatus for use in hot galvanizing and the like, an article to be brought into contact with molten zinc comprising a metallic body, said body having a coating of an enamel comprising a complex aluminum boro-silicate as the basis thereof together with boric-oxide and at least one metallic oxide on the surface of the body which comes into contact with the molten zinc to provide a heat conducting medium for protecting the body of the article from the action of the molten zinc. 100 105

In witness whereof, I hereunto set my hand.

WALLACE G. IMHOFF.